

# UNITED STATES PATENT OFFICE.

PIERRE GIRIN, OF PARIS, FRANCE, ASSIGNOR TO SOCIETE ANONYME DE COMMENTRY,  
FOURCHAMBAULT, & DECAZEVILLE, OF PARIS, FRANCE.

## ALLOY CONTAINING IRON, NICKEL, CHROMIUM.

1,422,096.

Specification of Letters Patent. Patented July 11, 1922.

No Drawing.

Application filed December 9, 1918. Serial No. 265,984.

To all whom it may concern:

Be it known that I, PIERRE GIRIN, a citizen of the Republic of France, residing in Paris, France, have invented certain new and useful Improvements in a new Alloy Containing Iron, Nickel, Chromium, of which the following is a specification.

Up to the present I am not acquainted, from the point of view of their application to chemical industries, with common alloys and metals which unite high mechanical qualities with a high resistance to the action of acids.

The present invention relates to alloys of iron, nickel, chromium, and manganese, to which may be added other metals, such alloy being susceptible of being cast, forged, rolled, drawn out, and otherwise worked and treated in the most complex manner, having a high mechanical resistance and a complete absence of fragility at all temperatures and practically unattacked by strong acids, especially organic acids, and equally by alkalis in solution or in fusion. Such an alloy may 25 comprise besides iron:

|           |     |        |           |
|-----------|-----|--------|-----------|
| Nickel    | 20  | to 25  | per cent. |
| Chromium  | 10  | to 15  | " "       |
| Manganese | 1   | to 2   | " "       |
| Carbon    | 0.2 | to 0.5 | " "       |

The compositions given above may undergo relatively important variations without the essential properties being sensibly modified; in particular the content in nickel may be carried even up to 40 per cent if we wish to best fulfil the conditions relating either to the elasticity or the coefficient of expansion of the alloy.

40 The manganese in the alloy insures satisfactory malleability.

The combined action of the nickel and of the chromium is to bring the iron into the condition  $\gamma$ . The alloy has then the mechanical advantages of ferro-nickels of 25 per cent nickel, with or without a small quantity of chromium, notably the property of being considerably deformed without fracture; but it presents relatively to this 50 last named alloy an absolute superiority as regards stability and resistance to corrosion.

The chromium has in effect the action of rendering any irreversible transformation

of the alloy absolutely impossible either at the most intense cooling ( $-200^\circ$ ) or by a 55 prolonged exposure to hot and moist gases; it suppresses, for example, the pittings and local changes which are an essential obstacle to the use in these conditions of ferro-nickel, with or without small additions of 60 chromium.

The addition of chromium in considerable quantities, such as 10 to 15 per cent, to a ferro-nickel reduces the corrosion of the metal by strong acids either hot or cold to 65 an insignificant amount.

By way of example, I may note that an alloy of the group defined above possesses at ordinary temperature a mechanical resistance of 60 to 80 kgs. per sq. mm., with 70 a coefficient of elongation of 30 per cent and a resilience which never falls below 25 kgms., as measured by the Guilloty apparatus on a sample of a 10 mm. cube having a rounded groove of a depth of 2 mm. In 75 cold concentrated nitric acid the loss of weight is of the order of 0.1 mg. per day per sq. cm., and in the same acid but at boiling temperature, of the order of 5 mg. per day per sq. cm.

80 This metal could be used advantageously in chemical industry for all the apparatus of complicated form or which is required to resist shocks whether due to high pressure (such as the worms, norias, centrifugal 85 pumps etc.) which are required to be in contact with acid materials. It would replace gold in the manufacture of inoxidizable pens.

Having thus described the nature of the 90 said invention and the best means I know of carrying the same into practical effect, I declare that what I claim is:—

An alloy of iron, nickel, chromium and manganese, containing nickel, 20 to 25 per 95 cent, chromium, 10 to 15 per cent, manganese, 1 to 2 per cent, carbon, 0.2 to 0.5 per cent, such alloy having, together with the mechanical qualities of the best steels, a high resistance to attack by strong acids, 100 organic acids and alkalis, in solution or in fusion.

In witness whereof, I have hereunto signed my name.

PIERRE GIRIN.